

June 24, 1958

J. COMPTON ET AL

2,840,446

PROCESS OF CYANOETHYLATING NATIVE COTTON FIBERS  
WITH AN AQUEOUS EMULSION OF SODIUM  
HYDROXIDE AND ACRYLONITRILE

Filed Oct. 10, 1955

6 Sheets-Sheet 1

FIG. 1



INVENTORS.

JACK COMPTON

BY CATESBY P. JONES

*Pearlie, Edmund, Malan, Bassett, Taylor*  
ATTORNEYS

June 24, 1958

J. COMPTON ET AL

2,840,446

PROCESS OF CYANOETHYLATING NATIVE COTTON FIBERS  
WITH AN AQUEOUS EMULSION OF SODIUM  
HYDROXIDE AND ACRYLONITRILE

Filed Oct. 10, 1955

6 Sheets-Sheet 2

FIG. 2



INVENTORS.  
JACK COMPTON  
BY GATESBY P. JONES  
*Pennie, Edwards, Morton, Pennie, et al.*  
ATTORNEYS

June 24, 1958

J. COMPTON ET AL

2,840,446

PROCESS OF CYANOETHYLATING NATIVE COTTON FIBERS  
WITH AN AQUEOUS EMULSION OF SODIUM  
HYDROXIDE AND ACRYLONITRILE

Filed Oct. 10, 1955

6 Sheets-Sheet 3

FIG. 3



INVENTORS.  
JACK COMPTON  
BY CATESBY P. JONES

*Pearce, Edwards, Morton, Brown, Taylor*  
ATTORNEYS

June 24, 1958

J. COMPTON ET AL

2,840,446

PROCESS OF CYANOETHYLATING NATIVE COTTON FIBERS  
WITH AN AQUEOUS EMULSION OF SODIUM  
HYDROXIDE AND ACRYLONITRILE

Filed Oct. 10, 1955

6 Sheets-Sheet 4

FIG. 4



INVENTORS.  
JACK COMPTON  
BY CATESBY P. JONES

*Penrie Edwards, Walter Bassett, Jr.*  
ATTORNEYS

June 24, 1958

J. COMPTON ET AL

2,840,446

PROCESS OF CYANOETHYLATING NATIVE COTTON FIBERS  
WITH AN AQUEOUS EMULSION OF SODIUM  
HYDROXIDE AND ACRYLONITRILE

Filed Oct. 10, 1955

6 Sheets-Sheet 5

FIG. 5

● % N. .014 lb. Na HO % O.D.P. ●  
○ % N. .021 lb. Na HO ○



INVENTORS.  
JACK COMPTON  
BY CATESBY P. JONES

*Pennington, Edmund, Martin, Bennett, Taylor*  
ATTORNEYS

June 24, 1958

J. COMPTON ET AL  
PROCESS OF CYANOETHYLATING NATIVE COTTON FIBERS  
WITH AN AQUEOUS EMULSION OF SODIUM  
HYDROXIDE AND ACRYLONITRILE

2,840,446

Filed Oct. 10, 1955

6 Sheets-Sheet 6

FIG. 6



FIG. 7



INVENTORS.

JACK COMPTON

BY CATESBY P. JONES

*Pennie, Edmund, Morton, Lawrence, Jr.*  
ATTORNEYS

1

2,840,446

## PROCESS OF CYANOETHYLATING NATIVE COTTON FIBERS WITH AN AQUEOUS EMULSION OF SODIUM HYDROXIDE AND ACRYLONITRILE

Jack Compton, Charlottesville, Va., and Catesby Perri-  
man Jones, Bethesda, Md., assignors to Institute of  
Textile Technology, Charlottesville, Va., a corporation  
of Virginia

Application October 10, 1955, Serial No. 539,486

6 Claims. (Cl. 8—120)

This invention relates to the reaction of acrylonitrile with cotton and has for its object the provision of improved cotton products and a process of reacting acrylonitrile with cotton fibers in the form of bulk fibers, yarns, or fabrics to improve the properties of the cotton while maintaining the natural structure of the fiber and most of the properties of ordinary cotton. Our invention provides an economical and practical process of producing our improved cotton products with a minimum loss of chemicals through washing, neutralizing and undesirable by-product formation. The improved cotton products of our invention are a partially cyanoethylated cotton, but they have the important distinction of retaining the natural fibrous form of native cotton fibers, and their crystallinity in a substantially unaltered state.

Several processes have been proposed heretofore for treating cellulose with aqueous solutions of sodium hydroxide and acrylonitrile to effect from a partial to a complete cyanoethylation, usually resulting in a soluble product, but, in any event, resulting in a product having a materially changed physical structure. Notwithstanding a considerable number of patents and other publications concerning the cyanoethylation of cotton and regenerated cellulose, namely rayon, there has not been any commercially successful process developed heretofore.

Our invention is based on several important discoveries we have made in an extensive investigation of the cyanoethylation of cotton through which we may control the conditions for reacting acrylonitrile.



with but a relatively small proportion of the cellulose giving cyanoethylcellulose which may be represented as Cell—O—CH<sub>2</sub>—CH<sub>2</sub>—CN. We have found that very desirable cotton products can be formed by effecting but a partial etherification of the cellulose molecule, resulting in but from 0.006 to 1.0 cyanoethyl group per anhydroglucose unit (equivalent to from 0.50 to 6.50% nitrogen based on the weight of cyanoethylated cotton). In the preferred and most advantageous embodiment of our invention, we control the conditions to combine but from 0.1 to 0.6 cyanoethyl group per anhydroglucose unit.

The following table shows the relationship between the cyanoethyl groups per anhydroglucose unit and the nitrogen content of the cyanoethylated cotton:

2  
Table A

|    | Percent N | Cyanoethyl Groups per Anhydro-Glucose Unit |
|----|-----------|--------------------------------------------|
| 5  |           |                                            |
|    | 0.50      | 0.060                                      |
|    | 0.62      | 0.074                                      |
|    | 0.77      | 0.092                                      |
|    | 1.20      | 0.146                                      |
| 10 | 1.64      | 0.220                                      |
|    | 1.77      | 0.202                                      |
|    | 1.89      | 0.236                                      |
|    | 2.40      | 0.306                                      |
|    | 3.08      | 0.417                                      |
|    | 3.16      | 0.405                                      |
|    | 3.80      | 0.515                                      |
|    | 4.30      | 0.595                                      |
| 15 | 4.85      | 0.691                                      |
|    | 5.24      | 0.760                                      |
|    | 6.52      | 1.020                                      |
|    | 9.80      | 1.820                                      |
|    | 13.00     | 3.000                                      |

- 20 Our invention is specifically directed to the treatment of "native" cotton because we aim to produce an improved cotton fiber and cotton is peculiarly suited to our process. By "native" cotton we mean natural cotton which has neither been changed chemically nor its molecular arrangement altered, although it may have been treated to remove gums, waxes and foreign matter. While cotton is a relatively pure form of cellulose, the fibers are considered to be formed of three distinct types of layers each having a different physical structure, consisting of 25 amorphous and crystalline components. Mild reaction conditions, such as the preferred cyanoethylation procedure herein described, are required to maintain this desirable fiber structure. In particular the relationship between the amorphous and crystalline components 30 should be maintained. One further characteristic of useful native cotton fibers is that the degree of polymerization of the cellulose varies from about 1500 to 4500 and in this respect it differs from viscose rayon which has a degree of polymerization of from about 150 to 450. 35 40 In general, all regenerated cellulosic fiber materials have a greater proportion of the amorphous component than native cotton and the crystalline component is characterized by having the mercerized cellulose molecular arrangement. Cotton thus has a different structural arrangement and responds differently than regenerated cellulose when treated with such chemicals as sodium hydroxide and acrylonitrile. Because of its structure, cotton is a very important textile material and our process maintains its structural identity. 45 50 For the cyanoethylation of cotton, we have discovered a very important relationship involving the concentration of sodium hydroxide in solution, the amount of sodium hydroxide solution applied to the cotton with the acrylonitrile, and the time and temperature of the reaction of 55 acrylonitrile with the cotton while in the presence of a solution of sodium hydroxide to effect the amount of cyanoethylation necessary to produce the improved cotton products. We can carry out our process in producing our improved cotton products without excessive loss 60 in sodium hydroxide and in by-product formation which results in a loss of acrylonitrile.

In accordance with the process of our invention, we apply to the cotton a mixture of an aqueous solution of sodium hydroxide and acrylonitrile, which mixture dur-

ing treatment is in a state of emulsion, and preferably by circulation of the emulsion over and through the cotton fibers. We may form the emulsion in any suitable way as by mechanically mixing the sodium hydroxide solution, a surface active agent such as Aerosol-OS (isopropyl naphthalene sodium sulfonate), and the acrylonitrile, and apply this emulsion to the cotton. An emulsion formed by mechanical agitation of an aqueous solution of sodium hydroxide and acrylonitrile may also be used as is described in our prior application, Serial No. 435,904, filed June 10, 1954, now abandoned. The emulsion may be formed, as therein described, by adding the sodium hydroxide solution to the acrylonitrile as it enters a circulating pump which in turn circulates the emulsion over the cotton very shortly after the emulsion is formed. Such a mechanically formed emulsion is not stable and separates quickly. By the use of a surface-active agent, such as Aerosol-OS, the emulsion may be stabilized.

In carrying out our invention, precautions must be taken to direct the addition of the cyanoethyl groups  $-\text{CH}_2-\text{CH}_2-\text{CN}$  without or with no appreciable hydrolysis to form carboxyethyl groups



In using the low sodium hydroxide concentrations in our process we avoid hydrolyzing the nitrile  $-\text{CN}$  to carboxyl  $-\text{COOH}$  and also neither depolymerize the crystalline cellulose nor increase the proportion of the amorphous fiber component.

Our invention provides improved cotton products derived from native cotton characterized by having the amorphous portion of the fibers combined with acrylonitrile in the form of cyanoethylcellulose while substantially all of the crystalline structure of the cotton fiber is retained. The amorphous portion has such an amount of combined acrylonitrile that the nitrogen content of the entire fiber varies from 0.50% to 6.5%.

The partially cyanoethylated cotton fibers of our invention are similar in appearance, hand, and processing characteristics to cotton, but differ primarily and significantly in that they are permanently resistant to micro-organism attack, such as cause mildew; more resistant to wet and dry heat degradation; more receptive to many dyes of all classes, including acid dyes; and more resistant to abrasion.

In our copending application, Serial No. 442,762 filed July 12, 1954, now Patent No. 2,786,258, we describe and claim our improved fibrous cotton product, and a process for treating cotton fibers with aqueous solutions of sodium hydroxide, preferably in a steeping process, and under the conditions described herein, but in the process of that application the presteepled cotton fibers are treated with liquid acrylonitrile containing some water. In the process of our copending application, Serial No. 435,903, filed June 10, 1954, now Patent No. 2,786,735, the presteepled cotton fibers are treated with acrylonitrile in the vapor phase.

We have discovered a significant relationship between the concentration of sodium hydroxide, the amount of water with respect to the cotton and the acrylonitrile, and the temperature and time of treatment of the cotton to form our improved cotton product efficiently, with a minimized loss of acrylonitrile through by-product formation. Our invention is based upon a control of the quantities of reactants and the conditions of treatment to form cyanoethylated cotton having the required nitrogen content and characteristic fibrous character of native cotton efficiently. The process of the invention comprises (1) the use of a relatively low concentration of sodium hydroxide in the aqueous solution which results in increased reaction efficiency, (2) the use of an accurately controlled quantity of water in the emulsion with acrylonitrile to achieve uniform reaction with the cotton and minimize by-product formation, (3) the control of temperature

and (4) a control of time in relation to the nitrogen content of the cotton.

One of the primary reaction variables is the sodium hydroxide concentration. This should be kept as low as practicable, preferably in the weight ratio of sodium hydroxide to cotton of from 0.005 to 0.10. The reaction efficiency, as used herein, is defined as the ratio of the theoretical amount of acrylonitrile required to give the found nitrogen content of the cyanoethylated cotton to the total amount non-recoverable, expressed as a percentage. The non-recoverable acrylonitrile includes the acrylonitrile fixed by reaction with the cellulose, that reacting with the water to form beta-beta'-oxydipropionitrile (ODP) and other by-products. There is also a significant relation between the water concentration in the emulsion and the temperature, the reaction efficiency increasing with a reduction in the water content, especially when this is accompanied by increasing temperatures.

Several variables affecting the nitrogen content of the cyanoethylated cotton include variations in the temperature and in the amount of sodium hydroxide based on the weight of the cotton. For example, with respect to the sodium hydroxide effect, the nitrogen content of the cotton can be increased from a mean of 2.48% to a mean of 3.02% when the weight ratio of sodium hydroxide to cotton is increased from 0.014 to 0.021. With respect to the temperature effect, the nitrogen content of the cotton can be increased from a mean of 2.52% to a mean of 2.98% by increasing the reaction temperature from 63° C. to 68° C. If the reaction time is constant, the two variables, sodium hydroxide content and reaction temperature can be changed individually or together to control the extent of cyanoethylation as indicated by the nitrogen content. Advantageously, the reaction temperature should be as high as possible and reaction time as short as possible.

In its complete aspects our invention comprises the circulation of an aqueous emulsion of sodium hydroxide solution in acrylonitrile while in contact with the fibers of native cotton in which the total water phase, representing from 50% to 150% of the weight of the cotton, contains from 0.50 to 10 percent of sodium hydroxide at a temperature of from 24° C. to 93° C. and for from 1 to 360 minutes to cyanoethylate preferentially the amorphous portion of the cellulose to such an extent that the cotton contains from 0.5 to 6.5% of nitrogen, the ratio of the weight of sodium hydroxide to the weight of the cotton being from 0.005 to 0.10.

In the accompanying drawings:

Figs. 1, 2 and 3 are curves showing the effects of variations in the water in the liquid phase at different temperatures and sodium hydroxide concentrations;

Figs. 4 and 5 are a series of curves showing the percentages of ODP with variations in the sodium hydroxide, temperature, time and water in the liquid phase;

Figs. 6 and 7 are a series of curves showing the effects of variations in the sodium hydroxide in the liquid phase, with variations in the sodium hydroxide based on the cotton, water in the liquid phase, and time.

The process of the invention may be carried out in any suitable kind of equipment in which the emulsion of the aqueous sodium hydroxide solution in acrylonitrile, at the proper temperature, is circulated in contact with the cotton for a sufficient time to effect the reaction resulting in cyanoethylation of the cotton. The Gaston County package dyeing machine which treats packages of yarn in kiers is one suitable kind of machine for practicing the invention. In the particular operations herein described, a Gaston County packaging machine containing 70 packages of cotton yarn in the two kiers were treated in each operation. The package weights were usually one-pound, but this varied slightly from run to run. By winding the cotton yarn on Davidson springs and compressing them to the maximum extent, it was possible to put as much as 98 pounds on the 70 packages. The ratio of the treating

components of the emulsion to cotton could thus be varied over a wide range. The following representative operation was carried out with 70 packages of cotton yarn and is typical of the other operations which were carried out under the variable conditions reported in the accompanying drawings.

To 530 pounds of acrylonitrile contained in a circulating tank connected to the two kiers, a mixture of 1 pound of sodium hydroxide and 0.5 pound of Aerosol-OS dissolved in 42 pounds of water was added. The mixture was then circulated through a centrifugal pump, while agitation was supplemented by the use of a Lightning mixer placed in the top of the circulating tank. After circulating for 30 minutes in this way at room temperature, an emulsion of the sodium hydroxide solution in the acrylonitrile was obtained. The two kiers of the package treating machine were then loaded with 67 pounds of cotton yarn containing 6 percent moisture in the usual manner and after closing the kiers the emulsion of sodium hydroxide solution in acrylonitrile was pumped through the packages at room temperature, 24° C., for 30 minutes. This resulted in a liquor to cotton ratio of 10.7 to 1. At the end of this time the temperature of the liquor, while being continuously circulated through the packages, was raised over a period of 5 minutes from 24° C. to 68° C. The rate of flow of the liquor through the packages was approximately 250 gallons per minute. The circulation was continued for 30 minutes, at 68° C., after which the liquor was cooled to room temperature and the sodium hydroxide neutralized with an aqueous phosphoric acid solution. The acrylonitrile remaining in the yarn in the kiers of the package machine was then removed by washing with water. It was found that about 90% of the acrylonitrile retained by the packages was removed by three charges of water weighing roughly 700 pounds each. These wash waters were collected and, with the spent acrylonitrile liquors from the reaction, subjected to flash distillation for recovery of the unreacted acrylonitrile. The yarn packages, after thorough washing in the package machine with water to remove all traces of acid and salts, were removed, centrifuged, and carried to a package drying unit, where warm air was blown through them until they were substantially dry. From the 7/1 cotton yarn treated in this instance, 81 pounds of cyanoethylated cotton yarn, containing 4.5% nitrogen, were obtained. Simultaneously, with the reaction of acrylonitrile with cotton, the acrylonitrile also reacted with part of the water present, so that 30 pounds of acrylonitrile went into by-product formation while 14 pounds of acrylonitrile were fixed on the yarn. This gave a ratio of acrylonitrile going into by-product formation to acrylonitrile fixed on the yarn of 2.1 to 1, or a reaction efficiency of 32%. The effective initial caustic concentration was calculated to be 2.1 percent and the ratio of caustic to cotton was 0.016.

In another example, 400 pounds of acrylonitrile containing 5.1 percent ODP were placed in a circulating tank connected to the kiers and a mixture of 3.65 pounds of sodium hydroxide and 0.5 pound of Aerosol-OS dissolved in 49 pounds of water added. The mixture was then circulated through a centrifugal pump while agitation was supplemented by use of a Lightning mixer placed in the top of the circulating tank. After agitating for 30 minutes in this way at room temperature, an emulsion of the sodium hydroxide solution was obtained. One of the two kiers of the package treating machine was then loaded with 38 pounds of yarn containing a 6 percent moisture in the usual manner, whereas the other kier was cut out of the system. This resulted in a liquor to cotton ratio of 10.1 to 1. After closing the charged kier, the emulsion of sodium hydroxide solution in acrylonitrile was pumped through the packages at room temperature, 24° C., for 30 minutes, reversing the direction of flow at 4-minute intervals. At the end of this time the

temperature of the liquor while being continuously circulated through the packages was raised over a period of 5 minutes from 24° C. to 38° C. The rate of flow of the liquor through the packages was approximately 250 gallons per minute. The circulation was continued for 30 minutes at 38° C., after which the liquor was cooled to room temperature and the sodium hydroxide neutralized with an aqueous phosphoric acid solution. The packages of 7/1 yarn after thorough washing and drying, as described above, weighed 45.4 pounds and upon analyzing were found to contain 4.3 percent nitrogen. The spent liquor from the reaction sampled at the completion of the reaction contained 10.9 percent ODP. Thus 16 pounds of acrylonitrile went into by-product formation, while 7.4 pounds were fixed to the yarn. This gave a ratio of acrylonitrile going into by-product formation to acrylonitrile fixed on the yarn of 2.2 to 1, or a reaction efficiency of 31 percent. It will be noted that the effective caustic concentration in this run was 7.1 percent in the water phase of the emulsion initially, and the ratio of caustic to cotton was 0.10.

A sample of yarn taken from the above run after the 30-minute circulation of the treating liquor at 24° C. was freed of caustic and acrylonitrile by acid neutralization and water washing. After drying the cyanoethylated yarn had a nitrogen content of 2.2 percent, indicating that the reaction proceeds fairly rapidly during the circulation period prior to raising the temperature to 38° C.

The foregoing typical operations were carried out many times with varying amounts of water in the liquid phase, varying sodium hydroxide to cotton ratios, varying temperatures and varying periods of treatment.

The curves of Figs. 1, 2 and 3 indicate that the water and sodium hydroxide approach and equilibrium between the liquid phase and the cotton during the first ten minutes of circulation. The water concentration of the liquid phase is reduced to about one-half its original amount while the sodium hydroxide concentration is reduced ten-fold during the first ten minutes of circulation. When the mixture contained 6 percent water at the beginning, the water content of the liquid phase approached the solubility limit of water in acrylonitrile at 24° C. (which was the approximate temperature maintained during cold circulation).

As the reaction temperature was increased, the water was dissolved in the liquid phase. In the series of experiments performed with 6 percent water in the liquid phase at the beginning, slightly more than 6 percent appeared after the reaction mixture was heated. This is probably caused either by water retained in the system or regain moisture in the yarn. With 8 percent water at the start, the liquid phase approached 8 percent water content as a limit during reaction. At 10 percent, the limiting factor for the water content during the reaction period was the solubility of water in acrylonitrile, so the water content of the liquid phase did not approach 10 percent in this series. Increasing the sodium hydroxide concentration from 0.014 lb. to 0.021 lb. per pound of cotton had no apparent effect upon the distribution of water between the yarn and liquor phases.

The operations show that the variable that has the most effect upon reaction efficiency appears to be the sodium hydroxide concentration and that it should be kept as low as possible for the desired nitrogen content of the yarn.

The data in Fig. 4 compare the rate of ODP formation for each operation. These data indicate that ODP formation is approximately linear with time. At 6 percent water in the liquid phase there is little difference in ODP formation when other reaction variables are changed, although the higher sodium hydroxide concentration is associated with the greatest ODP formation.

At 8 percent water, the effects of both temperature and sodium hydroxide upon ODP formation are shown,

If either reaction temperature or sodium hydroxide concentration is increased, the ODP formation is also increased.

At 10 percent water, it is apparent that the sodium hydroxide concentration has a greater effect upon ODP formation than reaction temperature; since the slopes of the lines comparing ODP formation at different sodium hydroxide concentrations are higher than those comparing different reaction temperatures.

In Fig. 5 the percentage nitrogen fixed to the yarn and the amount of ODP in the spent reaction liquor formed in each reaction is compared with the amount of water in the original reaction mixture. It is interesting to note that the nitrogen content of the yarn is decreased in most instances as the water in the reaction mixture is increased. This follows from the fact that the amount of sodium hydroxide per pound of cotton was held constant, and hence the actual sodium hydroxide concentration in the system was decreased as the amount of water introduced was increased.

The data in Figs. 6 and 7 show the effect of time of cold circulation upon the sodium hydroxide concentration of the liquid phase. Note that the sodium hydroxide concentration drops by a factor of ten during the first 5 minutes of cold circulation. The sodium hydroxide was absorbed most rapidly from the highest sodium hydroxide concentration.

It may be concluded that the rate and extent of cyanoethylation of cotton may be realized along with a minimum of ODP by-product formation by the proper control of the reaction variables of time, temperature, initial caustic concentration in the water phase of the caustic solution-acrylonitrile dispersion, and the related final ratio of caustic to cellulose as well as the concentration of the water phase in the acrylonitrile.

The one-step cyanoethylation process of the invention results in (1) less handling costs in the case of yarn treatment, (2) decreased by-product formation, (3) the use of water saturated acrylonitrile in the reaction, and (4) decreased the overall time for treatment. Each of these factors tends to improve the economics of the cyanoethylation process.

This application is a continuation-in-part of our patent application Serial No. 435,904, filed June 10, 1954, now abandoned.

We claim:

1. The process of treating native cotton fibers to effect but a partial cyanoethylation of the cellulose and retain the natural physical structure of the cellulose which comprises circulating in contact with said fibers an emulsion of an aqueous solution of sodium hydroxide in acrylonitrile at a temperature of from about 24° C. to 93° C. and in which the ratio of sodium hydroxide to cotton by weight varies from 0.005 to 0.100, and continuing the circulation until the cotton is combined with such an amount of acrylonitrile that the nitrogen content thereof varies for different reaction conditions from 0.5% to 6.5% based on the weight of the cyanoethylated cotton.
  2. The process of claim 1, wherein the emulsion is circulated over the cotton at normal room temperature.

for a time up to about 30 minutes and then the emulsion is circulated over the cotton at an elevated temperature up to 93° C.

3. The process of treating native cotton fibers to effect but a partial cyanoethylation of the cellulose and retain the natural physical structure of the cellulose which comprises circulating in contact with said fibers an emulsion of an aqueous solution of sodium hydroxide in acrylonitrile, said emulsion containing up to 12% of water with respect to the acrylonitrile and such an amount of sodium hydroxide that the ratio of sodium hydroxide to cotton varies from 0.005 to 0.10, the circulation being continued for a sufficient time to combine with the cotton such an amount of acrylonitrile that the nitrogen content thereof varies for different reaction conditions from 0.5% to 6.5% based on the weight of the cyanoethylated cotton without producing more than 10% oxydipropionitrile as a by-product in the spent liquor.

4. The process of claim 3, wherein the circulation is continued up to 20 minutes.

5. The process of treating native cotton fibers to effect but a partial cyanoethylation of the cellulose and retain the natural physical structure of the cellulose which comprises circulating in contact with said fibers an emulsion 25 of an aqueous solution of sodium hydroxide in acrylonitrile at a temperature of from about 63° C. to 79° C., the ratio of the weight of sodium hydroxide to the weight of cotton being from 0.005 to 0.10, said emulsion consisting principally of an aqueous solution containing from 30 0.5 to 10.0% of sodium hydroxide and said emulsion containing not over 12% of water, circulating the emulsion over said fibers until the cotton is combined with the acrylonitrile to such an extent that the nitrogen content thereof varies for different reaction conditions from 0.50 35 to 4.5% based on the weight of the cyanoethylated cotton.

6. The process of treating native cotton fibers containing both crystalline and amorphous cellulose which comprises reacting the cotton with an emulsion of an aqueous sodium hydroxide solution and acrylonitrile in which the 40 water phase contains from 0.5 to 10.0% of sodium hydroxide, the ratio of the weight of sodium hydroxide to the weight of the cotton being from 0.005 to 0.10, continuing the reaction at a temperature of from 62.8° C. to 79.4° C. until the amorphous portion of said fibers 45 are cyanoethylated to such an extent that the cotton contains from 0.50 to 4.5% of nitrogen based on the dry weight of the cyanoethylated cotton and in which substantially all of the original crystalline structure of the native cotton is retained, said cyanoethylated cotton having the appearance, hand and processing characteristics 50 of the native cotton, increased abrasion resistance, increased tensile strength, decreased moisture absorptivity, and increased affinity for acetate, vat and sulfur dyes.

**References Cited in the file of this patent**

UNITED STATES PATENTS

- 2,284,896 Hanford ----- June 2, 1942  
2,482,001 MacGregor ----- Sept. 13, 1949  
2,627,477 Downey ----- Feb. 3, 1953

UNITED STATES PATENT OFFICE  
CERTIFICATE OF CORRECTION

Patent No. 2,840,446

June 24, 1958

Jack Compton et al.

It is hereby certified that error appears in the printed specification of the above numbered patent requiring correction and that the said Letters Patent should read as corrected below.

Column 1, line 55, for "0.006" read --0.06--; column 8, line 59, list of references cited, under the heading "UNITED STATES PATENTS", for the patent number "2,482,001" read --2,482,011--.

Signed and sealed this 7th day of October 1958.

(SEAL)

Attest:  
KARL H. AXLINE

Attesting Officer

ROBERT C. WATSON  
Commissioner of Patents